

1

3,505,857  
ANALYSIS OF GASOLINE BLENDING  
COMPONENTS

Gilbert I. Jenkins, Ascot, England, assignor to The British Petroleum Company, Limited, London, England  
No Drawing. Filed Feb. 20, 1969, Ser. No. 801,186  
Claims priority, application Great Britain, Feb. 28, 1968,  
9,653/68  
Int. Cl. G01n 33/22

U.S. CL. 73—61

10 Claims

### ABSTRACT OF THE DISCLOSURE

The RON, MON, RVP and SG of a low olefin, lead free gasoline blending component are determined by measuring the percentage of the component in each of 12 specified chemical groups and applying regression equations.

This invention relates to the analysis of gasoline blending components and in particular to a chromatographic method of determining the Research Octane Number of certain gasoline blending components.

The method according to the invention is suitable for use with gasoline blending components (hereinafter called the "specified blending components") which contain only low concentrations of olefins and which are lead free. It is not applicable to blending components which contain a large proportion of olefins, e.g. blending components obtained by cracking. (Most finished gasolines cannot be analysed in accordance with the invention because they contain lead alkyl anti-knock agents and too great a proportion of olefins.)

The method according to the invention is particularly suitable for the analysis of the following four gasoline blending components:

### LIGHT STRAIGHT RUN GASOLINES

These are obtained by the distillation of crude petroleum and they consist predominantly of hydrocarbons which have 4-6 carbon atoms per molecule.

### CATALYTIC REFORMATES

These contain a large proportion of aromatics obtained from paraffins by dehydrogenation of cyclic paraffins and dehydrocyclisation of acyclic paraffins.

### MOTOR BENZOLES

These have a high concentration of benzene, e.g. 60-100% by volume, and they are often obtained from a non-petroleum source.

### ISOMERIZATES

These contain a large proportion of branched chain paraffins obtained by isomerization of straight chain paraffins.

As well as determining the Research Octane Number the method according to the invention can be used to determine the Reid Vapour Pressure, the Specific Gravity and the Motor Octane Number by a single experimental procedure. (It is pointed out that any one or any combination of this inspection data can be determined.)

The inspection data mentioned above, particularly the two octane ratings, require elaborate and time consuming procedures and a knowledge of the results is useful for controlling refinery plant and the method according to the invention makes the results available more quickly than conventional laboratory techniques. This increase in speed is an advantage to plant operators.

According to the invention a method of analysing a sample of a specified gasoline blending component comprises:

2

(a) Separating the sample into the following 12 groups,  
Group 1: n-butane and all compounds more volatile than  
n-butane,  
Group 2: all compounds less volatile than Group 1 and  
more volatile than Group 3,  
Group 3: n-pentane,  
Group 4: all compounds less volatile than Group 3 and  
more volatile than Group 5,  
Group 5: n-hexane,  
Group 6: all compounds less volatile than Group 5 and  
more volatile than Group 7,  
Group 7: benzene,  
Group 8: all compounds less volatile than Group 7 and  
more volatile than Group 9,  
Group 9: toluene,  
Group 10: all compounds less volatile than Group 9 and  
more volatile than Group 11,  
Group 11: all aromatic hydrocarbons whose molecule  
contains 8 carbon atoms (together with a few other  
compounds with boiling points in the same range),  
Group 12: all compounds less volatile than Group 11, and

(b) Determining the quantity of material contained in  
each of the twelve groups. (Percentage by weight is a  
convenient system of measurement but any other system  
which gives the relative concentrations can be used.)

The Research Octane Number, Reid Vapour Pressure,  
Specific Gravity and Motor Octane Number can be cal-  
culated from the relative quantities obtained above by  
suitable linear regression equations. All the coefficients  
and the constant term may be derived statistically by  
using data obtained from a sufficient number of samples.  
If desired certain coefficients can be derived from a  
knowledge of the properties of any pure compounds con-  
sidered. From time to time results obtained by the method  
according to the invention should be checked by tests  
carried out in the laboratory by conventional techniques  
and the regression equations up-dated when necessary.  
The calculation can be carried out either "by hand" or  
by computer; the latter is convenient for "closed loop"  
control.

According to a preferred embodiment of the invention  
the separation is carried out chromatographically. This  
technique is particularly suitable for "on-line" use since  
automatic chromatographs are commercially available.  
These give results in digital form and they can be con-  
nected to provide direct input into a computer. The  
chromatographic method is relatively rapid and it can  
provide a set of results about 20 minutes after the in-  
jection of the sample.

Furthermore a chromatograph can provide results at  
frequent intervals, e.g. it can provide one set of results  
every 40 minutes.

The 12 groups specified above give accurate results but,  
if desired, more accurate results can be obtained, at the  
expense of more complicated regression equation, by di-  
viding one or more of the groups specified above into two  
or more sub-groups. We will now give examples of such  
sub-division and, if desired, any one or more of these sub-  
divisions may be utilised.

### Group 1

This group could be split into two fractions namely,  
n-butane and the remainder of the group.

### Group 4

This group could be divided into two or three sub-  
groups namely, 2-methyl pentane, 3-methyl pentane (or  
these two combined in a single sub-group) and the re-  
mainder of the group.

**3**  
Group 6

This group could be divided into two sub-groups namely, methylcyclopentane and the remainder of the group.

Group 8

This group could be divided into from two to five sub-groups namely, 2-methyl hexane, 3-methyl hexane (or these two combined in a single sub-group), 2:2:4-trimethyl pentane, n-heptane and the remainder of the group. (In cases where the concentration of 2:2:4-trimethyl pentane and/or n-heptane are high it is preferable to create a separate sub-group for whichever compound has the high concentration, or two sub-groups if both have high concentrations. The compound with the low concentration, or both compounds if both have low concentrations, is conveniently comprised in the remainder.)

Groups 11 and 12

If desired individual aromatic compounds contained within these groups could be used as sub-groups which 20 contain a single compound. In some cases it may be desirable to use a sub-group which contains more than one compound, e.g. a sub-group which contains all the xylenes.

By way of example nine different gasoline blending components were chosen for analysis in accordance with 25 the invention.

A sample of each was separated chromatographically into the twelve groups defined above and the Research Octane Number (RON), Reid Vapour Pressure (RVP), Specific Gravity (SG) and Motor Octane Number 30 (MON) were obtained using the regression equations given in Table 1. (In these equations  $G_n$  is used to designate the percent by weight in the  $n$ th group.)

The experimental results are given in Table II which shows the percent by weight in each group for each 35 sample, the RON, RVP, SG and MON as calculated from these percentages and, for the sake of comparison the RON, RVP, SG and MON as obtained by conventional laboratory tests.

TABLE I

$$\begin{aligned} \text{RON} = & 103 - 0.093G_2 - 0.407G_3 - 0.173G_4 - 0.776G_5 \\ & + 0.088G_7 - 0.606G_8 + 0.070G_9 - 0.322G_{10} + 0.152G_{11} \\ & - 0.082G_{12} \end{aligned}$$

$$\text{RVP} = 2.6 + 1.14G_1 + 0.16G_2 + 0.135G_3 + 0.05G_4 + 0.05G_5$$

$$\begin{aligned} \text{SG} = & 0.88 + 0.00323G_1 - 0.00256(G_2 + G_3) - 0.00230G_4 \\ & - 0.00219G_5 - 0.00193G_8 - 0.00292G_{10} - 0.00065G_{11} \end{aligned}$$

$$\text{MON} = 23.7 + 0.83 \text{ RON} - 20 \text{ SG}$$

NOTE.—The last equation requires less calculation once RON and SG have been calculated. For cases where one of these is not calculated a complete regression equation for 50 MON can be obtained by substitution for RON and SG.

**4**

(a) Separating the sample into the following 12 groups, Group 1: n-butane and all compounds more volatile than n-butane,

Group 2: all compounds less volatile than Group 1 and more volatile than Group 3,

Group 3: n-pentane,

Group 4: all compounds less volatile than Group 3 and more volatile than Group 5,

Group 5: n-hexane,

Group 6: all compounds less volatile than Group 5 and more volatile than Group 7,

Group 7: benzene,

Group 8: all compounds less volatile than Group 7 and more volatile than Group 9,

Group 9: toluene,

Group 10: all compounds less volatile than Group 9 and more volatile than Group 11,

Group 11: all aromatic hydrocarbons whose molecule contains 8 carbon atoms (together with a few other compounds with boiling points in the same range),

Group 12: all compounds less volatile than Group 11,

(b) Determining the quantity of material contained in each of the twelve groups, and

(c) Calculating, from suitable regression equations which utilise the quantities determined in (b), at least one of the Research Octane Number, Reid Vapour Pressure, Specific Gravity, Motor Octane Number and a control parameter suitable for controlling a plant producing the gasoline blending component.

2. A method according to claim 1 in which Group 1 is split into two sub-groups, namely:

n-butane and

the remainder of the group.

3. A method according to claim 1, in which Group 4 is divided into two sub-groups namely:

2-methyl pentane together with 3-methyl pentane, and the remainder of the group.

4. A method according to claim 1, in which Group 4 is divided into three sub-groups namely:

2-methyl pentane,

3-methyl pentane, and

the remainder of the group.

5. A method according to claim 1, in which Group 6 is divided into two sub-groups namely:

methyl-cyclopentane, and

the remainder of the group.

TABLE II

|                              | Total catalytic reformate | Light catalytic reformate | Heavy catalytic reformate | Motor benzole | $C_5$ isomerize | $C_5/C_6$ isomerize | $C_6$ isomerize | Crude n-pentane | Straight run gasoline |
|------------------------------|---------------------------|---------------------------|---------------------------|---------------|-----------------|---------------------|-----------------|-----------------|-----------------------|
| G <sub>1</sub>               | 0.4                       | 1.9                       | 0.0                       | 0.0           | 0.3             | 0.5                 | 1.0             | 0.0             | 0.0                   |
| G <sub>2</sub>               | 8.4                       | 11.6                      | 0.3                       | 0.0           | 95.8            | 28.5                | 0.5             | 7.5             | 8.1                   |
| G <sub>3</sub>               | 6.4                       | 9.2                       | 0.3                       | 0.0           | 3.9             | 10.5                | 0.5             | 91.5            | 30.5                  |
| G <sub>4</sub>               | 11.4                      | 23.1                      | 1.2                       | 0.0           | 0.0             | 55.0                | 88.0            | 1.0             | 25.9                  |
| G <sub>5</sub>               | 4.2                       | 9.8                       | 0.4                       | 0.0           | 0.0             | 5.5                 | 9.0             | 0.0             | 20.1                  |
| G <sub>6</sub>               | 0.9                       | 2.5                       | 0.6                       | 0.2           | 0.0             | 0.0                 | 1.0             | 0.0             | 4.4                   |
| G <sub>7</sub>               | 6.8                       | 6.1                       | 0.3                       | 67.3          | 0.0             | 0.0                 | 0.0             | 0.0             | 0.5                   |
| G <sub>8</sub>               | 5.7                       | 25.1                      | 6.0                       | 1.3           | 0.0             | 0.0                 | 0.0             | 0.0             | 10.5                  |
| G <sub>9</sub>               | 22.0                      | 10.2                      | 18.1                      | 19.6          | 0.0             | 0.0                 | 0.0             | 0.0             | 0.0                   |
| G <sub>10</sub>              | 1.0                       | 0.4                       | 2.3                       | 0.2           | 0.0             | 0.0                 | 0.0             | 0.0             | 0.0                   |
| G <sub>11</sub>              | 23.7                      | 0.0                       | 34.0                      | 7.0           | 0.0             | 0.0                 | 0.0             | 0.0             | 0.0                   |
| G <sub>12</sub>              | 9.0                       | 0.0                       | 36.5                      | 2.6           | 0.0             | 0.0                 | 0.0             | 0.0             | 0.0                   |
| RON Expt.                    | 96.2                      | 73.6                      | 101.2                     | 110.4         | 92.5            | 83.6                | 80.6            | 65.0            | 64.0                  |
| RON Calc.                    | 95.6                      | 72.4                      | 101.4                     | 110.3         | 92.5            | 82.3                | 80.5            | 64.9            | 63.4                  |
| SG <sub>60/60° F</sub>       | 0.773                     | 0.682                     | 0.839                     | 0.874         | 0.625           | 0.649               | 0.663           | 0.625           | 0.659                 |
| SG <sub>60/60° F</sub> Calc. | 0.776                     | 0.696                     | 0.884                     | 0.872         | 0.624           | 0.640               | 0.652           | 0.624           | 0.657                 |
| MON Expt.                    | 85.0                      | 72.5                      | 9.0                       | 99.8          | 88.0            | 81.6                | 80.4            | 71.0            | 62.5                  |
| MON Calc.                    | 87.5                      | 69.9                      | 91.2                      | 97.8          | 88.0            | 79.2                | 77.5            | 65.1            | 63.2                  |
| RVP Expt.                    | 6.3                       |                           |                           |               | 19.6            |                     |                 | 15.9            |                       |
| RVP Calc.                    | 6.1                       |                           |                           |               | 18.8            |                     |                 | 16.2            |                       |
| SG <sub>60/60° F</sub> Expt. | 0.773                     | 0.682                     | 0.839                     | 0.874         | 0.625           | 0.649               | 0.663           | 0.625           | 0.659                 |

I claim:

1. A method of analysing a sample of a low olefin content, lead free gasoline blending component which comprises:

6. A method according to claim 1, in which Group 8 is divided into two sub-groups namely:

2-methyl hexane together with 3-methyl hexane, and the remainder of the group.

7. A method according to claim 6, in which Group 8 is divided into four sub-groups namely:

2-methyl hexane together with 3-methyl hexane,  
2:2:4-trimethyl pentane,  
n-heptane, and  
the remainder of the group.

8. A method according to claim 1, in which there is an additional sub-group which contains all the xylenes.

9. A method according to claim 1 in which the separation is carried out chromatographically.

10. A method according to claim 1, in which stage (c) uses linear regression equations.

#### References Cited

#### UNITED STATES PATENTS

3,438,242 4/1969 Ayers et al. ----- 73--23.1

LOUIS R. PRINCE, Primary Examiner

J. W. ROSKOS, Assistant Examiner

UNITED STATES PATENT OFFICE  
CERTIFICATE OF CORRECTION

Patent No. 3,505,857

Dated April 14, 1970

Inventor(s) Gilbert Ivor Jenkins

It is certified that error appears in the above-identified patent and that said Letters Patent are hereby corrected as shown below:

Table II, left-hand column, fifteenth line counting from "G1" as line 1, - for "SG60/60°F" read --SG 60/60°F Expt--;

Table II, column headed "Heavy Catalytic Reformate", line 17, captioned "MON Expt" - for "9.0" read --90.0--;

Table II, delete the last line; and

Column 4, line 18, - for "whole" read --whose--.

SIGNED AND  
SEALED

SEP 29 1970

(SEAL)

Attest:

Edward M. Fletcher, Jr.

Attesting Officer

WILLIAM E. SCHUYLER, JR.  
Commissioner of Patents